

## UNITED STATES PATENT OFFICE

ALADAR PACZ, OF EAST CLEVELAND, OHIO

## COATING ZINC AND CADMIUM

No Drawing.

Application filed May 28, 1927. Serial No. 195,140.

This invention relates to the coating of metals either for preservative or decorative purposes and has for its object the provision of a simple, convenient, and inexpensive process whereby zinc and cadmium can be provided with a thin adherent coating which is permanent and non-corrodible under all ordinary conditions, which is artistic and attractive to the eye when left naked, and which constitutes a satisfactory and enduring foundation for paint, enamel and other coatings; the provision of a process which shall be rapid and economical and which does not require the employment of wires, electric contacts, and electric potential; the provision of a simple process whereby coatings of different colors can be controllably produced; while further objects and advantages of the invention will become apparent as the description proceeds.

It is well known that zinc and cadmium are difficult metals to coat or color economically since the usual quickly applied coatings, both metallic and non-metallic, fail to adhere successfully thereto; and while articles of pure zinc and cadmium are quite rare, articles having a protective coating of those metals are very common, as well as certain alloys which contain the same and as a result exhibit certain chemical and electrical peculiarities commonly associated with these substances.

My invention is based upon the peculiar properties of certain molybdenum compounds, and consists essentially in depositing upon the surface of the article to be coated or colored an adhering coating of substantial density and hardness consisting apparently of one or more of the lower oxides of molybdenum formed thereon in situ. However, a pure solution of the molybdenum compound is not sufficient but the addition of certain other substances is necessary to produce the results in view.

In the performance of my said invention I subject the articles to the action of a solution containing a soluble molybdate, and other substances which accelerate and intensify the action thereof. This is preferably effected by immersing the articles bodily

in a solution of the requisite composition until the desired coating is obtained, although I do not exclude spraying, painting, etc. The molybdate used is preferably that of ammonium and the strength of the solution is preferably from about  $\frac{1}{2}\%$  to, say, 2% of ammonium molybdate. This material alone, at least in the cold and without electrical potential, is too slow in action at least for yielding dark coatings.

The presence of different acid radicals accelerates and intensifies the action. Of the many scores of substances I have tested the best results I have so far achieved have been with sulphuric acid in the form of ammonium sulphate, although I do not limit myself thereto since there may be other substances which will produce equivalent results. I prefer to employ an amount of this activating material in excess of the molybdate.

The solution is employed either neutral or acid (but not ammonical) either hot or cold. One advantage of my process is the ability to use ordinary room temperatures, although raising the temperature is permissible and produces even faster action. The longer the treatment the darker the color; the coating passes through the yellows, blues, reds, to a final black, and any desired color can be retained merely by stopping the treatment. Generally the treated article is finished merely by rinsing, although a coating of paint or enamel can be applied if desired and adheres better than to the naked metal.

Having thus described my invention what I claim is:

1. The process of coating articles consisting at least superficially of zinc or cadmium which contains the step of subjecting them to the action of a solution containing a water soluble molybdate and a sulphuric acid compound.

2. The process of coating articles consisting at least superficially of zinc or cadmium which contains the step of subjecting them to the action of a solution containing ammonium molybdate and ammonium sulphate.

3. A dipping solution for zinc and cad-

mium articles containing ammonium molybdate and ammonium sulphate.

4. A dipping solution for zinc and cadmium articles containing a soluble molybdate and a sulphuric acid compound.

5. A non-alkaline dipping solution for zinc and cadmium articles containing a soluble molybdate and a second soluble salt, such second salt being one which is not alkaline and does not precipitate molybdenum.

10 In testimony whereof I hereunto affix my signature.

ALADAR PACZ.

mium articles containing ammonium molybdate and ammonium sulphate.

4. A dipping solution for zinc and cadmium articles containing a soluble molybdate and a sulphuric acid compound.

5. A non-alkaline dipping solution for zinc and cadmium articles containing a soluble molybdate and a second soluble salt, such second salt being one which is not alkaline and does not precipitate molybdenum.

10 In testimony whereof I hereunto affix my signature.

**ALADAR PACZ.**

**CERTIFICATE OF CORRECTION.**

**Patent No. 1,784,106.**

**Granted December 9, 1930, to**

**ALADAR PACZ.**

It is hereby certified that error appears in the printed specification of the above numbered patent requiring correction as follows: Page 1, lines 69 to 71, strike out the words and period "I prefer to employ an amount of this activating material in excess of the molybdate."; same page, line 78, strike out the words "the treatment"; and that the said Letters Patent should be read with these corrections therein that the same may conform to the record of the case in the Patent Office.

Signed and sealed this 3rd day of February, A. D. 1931.

**(Seal)**

**M. J. Moore,  
Acting Commissioner of Patents.**

**CERTIFICATE OF CORRECTION.**

**Patent No. 1,784,106.**

**Granted December 9, 1930, to**

**ALADAR PACZ.**

**It is hereby certified that error appears in the printed specification of the above numbered patent requiring correction as follows: Page 1, lines 69 to 71, strike out the words and period "I prefer to employ an amount of this activating material in excess of the molybdate."; same page, line 78, strike out the words "the treatment"; and that the said Letters Patent should be read with these corrections therein that the same may conform to the record of the case in the Patent Office.**

**Signed and sealed this 3rd day of February, A. D. 1931.**

**(Seal)**

**M. J. Moore,  
Acting Commissioner of Patents.**